

## UNITED STATES PATENT OFFICE

IZADOR J. NOVAK, OF BRIDGEPORT, CONNECTICUT, ASSIGNOR TO THE RAYBESTOS COMPANY, OF BRIDGEPORT, CONNECTICUT, A CORPORATION OF CONNECTICUT

## SOLUBLE GILSONITE AND METHOD OF MAKING SAME

No Drawing.

Application filed July 26, 1929. Serial No. 381,405.

This invention relates to a method of producing a highly soluble gilsonite and a smooth, substantially sediment-free solution of the same.

It is well known that commercial gilsonite is very difficult to completely dissolve in the ordinary solvents such as gasoline or benzol unless, for instance, it is refluxed with these solvents at a high temperature. This 10 is probably due to the fact that gilsonite is highly colloidal and, therefore, tends to resist complete smooth solution.

With ordinary straight run gasoline and a gilsonite having a melting point of approximately 300° F. (ball and ring method) and ash of 0.2%, the maximum amount of gilsonite which enters the solvent, even when finely ground, is about 70 to 75%. It is slightly higher with benzol—80 to 90%. In both 20 cases, however, there is a considerable proportion which never goes into solution and further, most of the material in solution is still colloidal and swelled rather than dissolved and, therefore, is poorly suited as a 25 saturating material for brake linings for instance, where a considerable proportion of colloidal material is left on the surface when impregnation is attempted.

I have found that, by melting gilsonite 30 such as described above and holding it slightly above the temperature at which it is comparatively fluid, which may be, say, 325-400° F., for a period of one-half hour, more or less, the gilsonite is rendered extremely soluble 35 in both gasoline and benzol without material lowering of the original melting point. As a matter of fact, in most cases, no lowering is observed. After cooling, I find that such a previously melted gilsonite goes easily and 40 quickly into solution in gasoline and benzol or other similar or related solvents, leaving no appreciable residue except the inorganic matter which was contained.

After months of standing, such solutions in 45 gasoline have shown no appreciable sedi-

ment and are smooth and homogeneous. Further, it quickly and thoroughly saturates, for instance, woven asbestos-covered wire tape without leaving sediment on the surface indicating that the colloidal characteristics 50 of the untreated gilsonite have been very much reduced.

By the term gilsonite I wish to indicate asphaltites having a fusing point over 250° F. and a specific gravity between 1.05 and 55 1.12, fixed carbon 10-25%, solubility in carbon bisulfide greater than 96%. This is intended to include certain of the glance pitches which are so close in physical properties to true gilsonite that they are or may be 60 used for the same purpose.

I am aware that it is customary to make certain varnishes by combining gilsonite with natural gums and drying oils at high 65 temperatures whereby the gilsonite becomes truly soluble, but the intent of this invention is to produce a truly soluble gilsonite per se and not a combination with oils.

I claim as my invention:

1. A method for rendering gilsonite substantially completely soluble in gasoline and like solvents and for reducing the colloidal characteristics thereof which comprises melting the gilsonite by heating in the absence of the solvent and holding the same at a temperature slightly above its melting point for a time period sufficient to induce substantially 75 complete solubility when mixed with the solvent.

2. A method for rendering gilsonite substantially completely soluble in gasoline and like solvents and for reducing the colloidal characteristics thereof which comprises melting the gilsonite by heating in the absence of the solvent and holding the same at a temperature of 325° F. to 400° F. for at least one-half hour. 85

3. A process for producing a substantially complete solution of gilsonite in gasoline which comprises melting the gilsonite by 90

heating in the absence of the gasoline and holding the same at a temperature slightly above its melting point for a time period sufficient to induce substantially complete solubility in gasoline, and subsequently dissolving the thus treated gilsonite in gasoline.

4. A process for producing a substantially complete solution of gilsonite in gasoline which comprises melting the gilsonite by heating in the absence of the gasoline and holding the same at a temperature of 325° F. to 400° F. for at least one-half hour, and subsequently dissolving the thus treated gilsonite in gasoline.

In testimony whereof I affix my signature.

IZADOR J. NOVAK.

20

25

30

35

40

45

50

55

60

65